

## UNITED STATES PATENT OFFICE

2,336,087

## TEXTILE OIL

Alfred C. Goodings and Harry B. Marshall, Toronto, Ontario, Canada, assignors to Ontario Research Foundation, Toronto, Ontario, Canada

No Drawing. Application July 11, 1942,  
Serial No. 450,631

9 Claims. (Cl. 252—8.6)

This invention relates to improvements in textile oils.

Oil is used in the manufacture of textile materials, particularly in the carding and spinning of woollen and worsted yarns. This oil which is added to facilitate the manipulation of the fibres is subsequently removed by scouring before the cloth is dyed and finally finished ready for the retail market.

To be satisfactory for textile use, an oil must conform to certain definite requirements and therefore must possess certain definite properties. For example, it must not oxidise readily nor develop rancidity; it must not attack the card wires or other metal parts of the machines; it must have adequate lubricating properties, be completely liquid at ordinary working temperatures and of suitable viscosity; it must be readily removed from the textile material by simple scouring procedures. The oils which have been favoured for use in textile operation as conforming most closely to all requirements have been certain triglyceride oils of which olive oil has been regarded as the best. Mineral oils on the other hand have not been found satisfactory for textile use chiefly because of the difficulty or impossibility of removing them from wool by conventional scouring methods.

Mineral oils do, however, possess many properties which conform in a highly desirable manner to the requirements of an ideal textile oil, and, in addition, their availability and low cost relative to olive oil render very attractive any possibility of using them for textile purposes. Indeed the one bad feature associated with refined mineral oil (poorly refined oils have other disadvantages) is the serious difficulty experienced in its removal by scouring from the wool cloth made from yarns to which it has been applied. That this difficulty is a very real one can be readily illustrated by the results of experiments in which two samples of wool cloth were oiled with 10% by weight of olive oil in one case and 10% by weight of a mineral oil in the other and subjected to identical scouring procedures. The oil remaining in the fabrics after the scouring was subsequently determined and the following figures show this residual oil content as a percentage of the weight of oil originally present on the cloth before the scouring operation.

Residual oil left in the cloth, per cent

|             |      |
|-------------|------|
| Olive oil   | 7.6  |
| Mineral oil | 85.0 |

55

5 The problem of overcoming the difficulty encountered in the removal of mineral oil from wool and the rendering of such oil satisfactory for use in textile operations has been the subject of investigation, and as a result it has been found that the addition of small percentages of certain partially esterified polyhydroxy compounds could completely modify the scouring properties of mineral oil and render it the equivalent of olive oil in this regard. The partially esterified polyhydroxy compounds which were of particular interest were the monoglycerides and diglycerides. Although a number of these compounds had the desired influence in rendering mineral oil removable by scouring, from a practical point of view only those are of value which combine this efficiency with an ability to stay completely blended with the mineral oil. In other words, most otherwise suitable mono- and di-glyceride compounds segregate and separate out in greater or less degree from the mineral oil on standing, particularly at low temperatures. It was necessary therefore to develop liquid compounds which would remain properly blended under all conditions to be met in transportation, storage and normal use. This was achieved through the preparation of diglycerides having one of the acid chains consist of a short, rather than a long, aliphatic acid. A typical suitable 10 diglyceride was found to be coconut-acetic di-glyceride. The use of such compounds containing a short aliphatic acid chain along with a longer aliphatic acid in the diglyceride is described in United States Patent No. 2,238,882, 15 April 22, 1941.

15 Since the outbreak of the present hostilities and particularly during the past six months, a serious shortage of the compounds necessary to the preparation of the diglycerides of the type 20 described in United States Patent 2,238,882 has arisen. The object of the present invention, therefore, is to produce compounds having characteristics similar to those described in the above 25 mentioned patent which can be made from available materials.

25 This object has been attained by the use of naphthenic acid either to replace the short-chain aliphatic acids described in the above patent, or by the use of naphthenic mono-ester or di-ester 30 of a polyhydric alcohol instead of the di-esters described in said patent.

30 We have found that the monoglyceride and di-glyceride of naphthenic acid when mixed with mineral oil not only render the mineral oil removable by scouring, but also remain blended

with the oil without undesirable separation. The naphthenic mono- and diglycerides may be prepared in a known manner by reacting naphthenic acid with glycerol. Instead of glycerol other polyhydric alcohols such as erythritol or mannitol may be partially esterified with naphthenic acid to form naphthenic mono-esters and di-esters. The naphthenic mono-ester of glycol may also be used.

We have also found that a satisfactory scouring compound may be produced by reacting naphthenic acid with the mono-ester of long-chain aliphatic acids such as the constituent acids of coconut oil, lard oil, neatsfoot oil or oleic acid. For example lard oil may be changed from a triglyceride to a monoglyceride by reacting with glycerol, and the monoglyceride subsequently reacted upon with the appropriate quantity of naphthenic acid to give a di-glyceride of lard oil and naphthenic acid.

Partial esters of polyhydric alcohols can be prepared using naphthenic acids, the following being an illustration of a suitable method in which the polyhydric alcohol is glycerol.

(1) *Preparation of the naphthenic mono-ester of glycerol*

92 parts of glycerol and 250 parts by weight of the naphthenic acids are heated together with vigorous stirring in an atmosphere of nitrogen. The use of an atmosphere of nitrogen is to obviate the presence of oxygen and so prevent oxidation and an undue darkening in the colour of the product. The water which is formed in the reaction is distilled off and removed from the reaction chamber. The temperature is slowly raised during the reaction from about 180° C. to 230° C. to keep the water produced distilling off at a fairly uniform rate. The reaction is normally complete in four hours. Subsequent treatment of the product with 2-3% charcoal at about 100° C. is effective in removing objectionable odours which are associated with the crude naphthenic acids, and also improves the colour.

(2) *Preparation of the naphthenic di-ester of glycerol*

92 parts of glycerol and 500 parts by weight of the naphthenic acids are heated together with vigorous stirring in an atmosphere of nitrogen. The water produced by the reaction is kept distilling off at a fairly uniform rate by slowly raising the temperature from about 180° C. to 230° C. throughout the four hours required to carry out the completed preparation. Subsequent treatment of the product with 2-3% charcoal at 100° C. is an advantage to remove objectionable odours associated with crude naphthenic acids as well as to improve the colour of the product.

Mixed di-esters of glycerol can also be prepared using naphthenic acids in conjunction with long chain fatty acids such as are contained in lard oil. The following is a description of a di-ester of glycerol made from lard oil, glycerine and naphthenic acids.

(3) *Preparation of a mixed di-ester of glycerol (lard oil-naphthenic diglyceride)*

The preparation is carried out in two stages,

(a) Lard oil monoglyceride is first formed by the reaction of 2610 parts of lard oil and 600 parts by weight of glycerine with the addition of 4.5 parts of sodium hydroxide as catalyst. The materials are heated together with good agitation for 3 to 4 hours at 210° C. in the presence of an

atmosphere of nitrogen. No water is evolved in this reaction.

(b) The lard oil monoglyceride formed in (a) is allowed to react with naphthenic acids in the proportion of 351 parts by weight of the monoglyceride to 250 parts of the naphthenic acids. The materials are heated together with rapid stirring in a current of nitrogen, and the water evolved in the reaction is carried off. The temperature is gradually raised throughout the reaction from about 200° C. to 230° C. to keep the water distilling over at a steady rate. A point is finally reached at which no further water is formed, after which the reaction is complete. The time required to complete the reaction is about four hours. Subsequent treatment of the product with 2-3% charcoal is an advantage to remove objectionable odours associated with crude naphthenic acids and also for purposes of improving the colour of the product.

The quantity of these various compounds which is to be added to mineral oil to render it desirable for textile use is between 5% and 20%, a preferred quantity being 10% to 15%. The effectiveness of their addition to mineral oil on its ease of removal by scouring can be illustrated by the following table of results. In all cases wool fabric was oiled with 10% of its weight of oil. The fabric was then scoured under controlled conditions identical for each oil tested, and the oil left in the fabric subsequently determined. This residual oil is expressed as a percentage of the original weight of oil present on the wool before scouring. For comparison, results using olive oil, and mineral oil without any addition agent are included. The scouring was carried out in an aqueous solution of soap and soda-ash.

|                                                     | Residual oil left in the cloth, per cent |
|-----------------------------------------------------|------------------------------------------|
| 40 Olive oil                                        | 7.6                                      |
| 100% mineral oil                                    | 85.0                                     |
| 90% mineral oil+10% lard oil-naphthenic diglyceride | 19.1                                     |
| 85% mineral oil+15% lard oil-naphthenic diglyceride | 8.3                                      |
| 90% mineral oil+10% naphthenic mono-glyceride       | 12.5                                     |
| 85% mineral oil+15% naphthenic mono-glyceride       | 7.1                                      |
| 50 90% mineral oil+10% naphthenic diglyceride       | 20.0                                     |
| 85% mineral oil+15% naphthenic diglyceride          | 10.5                                     |

Suitable mineral oils for use in the present invention are preferably of the following general characteristics, these being given for example only and without intending to preclude reasonable variation.

Table I

|                                          | General range | Preferred range |
|------------------------------------------|---------------|-----------------|
| 65 Gravity, A. P. I.                     | 23-36         | 25-32           |
| Viscosity (Saybolt Universal at 100° F.) | 50-250        | 125-175         |
| Pour point                               | 0-50          | 25-35           |

Naphthenic acid is a product obtained in the refining of petroleum. More strictly, commercial naphthenic acid obtained in the course of petroleum refining is not a single chemical compound but a mixture of acids. For industrial uses it is customary to use this mixture of crude acids or separate fractions of the same. It is this commercial form of naphthenic acids, which

is comparatively cheap and plentiful, which we employ in the formation of partially esterified glycerides containing naphthenic acid.

Although naphthenic acids are very complex in their nature and scientific knowledge on the subject is limited, refined naphthenic acids are believed to consist of both mono- and bi-cyclic compounds built from a 5-membered ring, that is they are carboxylic acid derivatives of cyclopentane. A formula of one of the simplest naphthenic acids is as follows:



The naphthenic glycerides may be used in combination with triglycerides in the same manner as the diglycerides mentioned in the aforesaid United States Patent No. 2,238,882.

What we claim as our invention is:

1. A textile oil comprising about 80% to 95% of a mineral base oil having a viscosity within the approximate range of 50 and 250 seconds Saybolt Universal at 100° F. and containing as a scouring agent about 5% to 20% of a partial ester of a naphthenic acid and a polyhydric alcohol.

2. A textile oil comprising about 80% to 95% of a mineral base oil having a viscosity within the approximate range of 50 and 250 seconds Saybolt Universal at 100° F. and containing as a scouring agent about 5% to 20% of the mono-ester of polyhydric alcohol and naphthenic acid.

3. A textile oil comprising about 80% to 95% of a mineral base oil having a viscosity within the approximate range of 50 and 250 seconds Saybolt Universal at 100° F. and containing as a scouring agent about 5% to 20% of the di-ester of polyhydric alcohol and naphthenic acid.

4. A textile oil comprising about 80% to 95% 40

of a mineral base oil having a viscosity within the approximate range of 50 and 250 seconds Saybolt Universal at 100° F. and containing as a scouring agent about 5% to 20% of a di-ester of a polyhydric alcohol of at least three hydroxy groups with a long chain fatty acid and naphthenic acid.

5. A textile oil comprising about 80% to 95% of a mineral base oil having a viscosity within the approximate range of 50 and 250 seconds Saybolt Universal at 100° F. and containing as a scouring agent about 5% to 20% of naphthenic monoglyceride.

6. A textile oil comprising about 80% to 95% of a mineral base oil having a viscosity within the approximate range of 50 and 250 seconds Saybolt Universal at 100° F. and containing as a scouring agent about 5% to 20% of naphthenic acid diglyceride.

7. A textile oil comprising about 80% to 95% of a mineral base oil having a viscosity within the approximate range of 50 and 250 seconds Saybolt Universal at 100° F. and containing as a scouring agent about 5% to 20% of the di-ester of glycerol with a long chain fatty acid and naphthenic acid.

8. A textile oil comprising about 80% to 95% of a mineral base oil having a viscosity within the approximate range of 50 and 250 seconds Saybolt Universal at 100° F. and containing as a scouring agent about 5% to 20% of lard oil-naphthenic diglyceride.

9. A textile oil comprising about 80% to 95% of a mineral base oil having a viscosity within the approximate range of 50 and 250 seconds Saybolt Universal at 100° F. and containing as a scouring agent about 5% to 20% of oleic naphthenic diglyceride.

ALFRED C. GOODINGS.  
HARRY B. MARSHALL.